

May 2, 1939.

C. G. FINK ET AL.

2,156,262

PROCESS OF TREATING METAL ARTICLES TO ALLOY CONSTITUENT METALS

Filed Dec. 27, 1932



Colin G. Fink and Pinus Deren, INVENTORS

BY  
Gustave R. Thompson, ATTORNEY

## UNITED STATES PATENT OFFICE

2,156,262

PROCESS OF TREATING METAL ARTICLES  
TO ALLOY CONSTITUENT METALS

Colin G. Fink and Pincus Deren, New York, N. Y.

Application December 27, 1932, Serial No. 648,870

16 Claims. (Cl. 148—7)

This invention relates to a process of treating metal articles, to alloy constituent metals, and provides improvements therein.

Roberts-Austen (*Philosophical Transactions, Royal Society of London*, 1897, Series A, 187 p. 383) reviews the writings and work of scientists from the time of Pliny, on the subject of the diffusion of metals, (and also of matter) and states that previous investigators had reported that "alloys might be formed by placing carefully-cleaned pieces of two constituent metals in juxtaposition and heating them to the melting point of the alloy to be formed, which was, in some cases 150° below the melting point of the more fusible of the two metals". Looking backward, this article of Roberts-Austen assumes the rank of a classic, and in it may be perceived an adumbration of the entire modern achievements base on the emissivity of matter. In the experiments reported by Roberts-Austen, contrary to the present invention, the heats were maintained for long periods of time, thirty-one days, ten days, thirty days, twenty-nine days, forty-one days, four days, ten days, six days, as compared with 25 minutes according to the present invention, and the resulting alloys were non-uniform, the proportion of the two constituents varying progressively from the line of contact of the two metals.

Despite the scientific facts and data given by Roberts-Austen and many patents and publications which have since issued, we are unaware of any practical application thereof having been made in overcoming the difficulties in the production of refractory and resistant alloy articles which have come into commercial use in the last twenty-five years or thereabout.

Refractory alloys, such as the alloys, iron and nickel, iron and chromium, nickel and chromium, iron, nickel and chromium, etc., are difficult and costly to work from an ingot into shaped articles. Even simple articles, such as wire, strips, sheets, etc., are difficult and costly to so manufacture.

The present invention provides an improved process by which alloying (in whole or in part) may be effected of constituent metals of articles which are electroformed of two or more metals, or formed of a metal amenable to metal-working and electroplated, without destroying the form of the article. The alloying according to the present process may be effected in a very short time; minutes as compared with hours according to other processes heretofore used (such as "chromizing" and so-called "heat-treatment" processes) and may be carried on in air, or in a

reducing or non-oxidizing atmosphere in an ordinary manner.

According to our process, an article as a wire, rod, sheet, strip, shell, etc., is electroformed, or is formed of a metal which is readily worked, iron, nickel, copper, molybdenum, etc., or a readily workable alloy, (or an article already so formed), is coated with an electrodeposit of the metal to be alloyed therewith, and then heated to a temperature where the immediate faces of the metals in contact are molten or virtually so, which is at about the eutectic of the metals in contact, and above. The heating may be, and preferably is, carried out in two stages. In the first stage, the coated metal may be heated to a temperature at which a superficial layer of oxide is formed on the outer metal, which oxide layer serves to protect the metal beneath the oxide against the much more rapid oxidation which would take place were the article heated initially to the higher temperature used in the second heating stage. Some diffusion of the coating metal into the metal beneath it may take place. In the second heating stage, the temperature is raised to about the eutectic melting-point, or above where rapid diffusion and alloying of the metals occurs. At this high temperature excessive consumption of the coating metal by oxidation is defeated by the rapid diffusion and alloying of said coating metal with the underlying metal.

Contrary to what might be expected, the formed article does not lose its form when heated at or above the melting point of the eutectic, the probable explanation being that at any one instant the composition of the eutectic only exists at a line within the body of the article, the composition maintaining its solid form on each side of said line. Therefore, if the component metals are greater or less than the proportions forming the eutectic, the article will not melt, even though it be heated to a temperature at or above the temperature at which the eutectic melts.

The use of a reducing or non-oxidizing atmosphere, such as generally understood, around the articles during heating, while it does not prevent oxidation at the high temperatures employed in our process, reduces the consumption of the coating metal by oxidation, and its use is hence preferred.

While we have spoken of the temperature of the eutectic of the alloy as the temperature to which the constituent metals of the starting articles is to be heated in effecting a union thereof to form the alloy layer or band having a definite alloy or eutectic composition, nevertheless in

practice temperatures which vary somewhat from the temperatures of the melting points of the eutectics given in scientific treatises and tables are employed. A precise rule for all cases cannot be given. There is some empiricism in ascertaining the operating temperature. Certain limitations in the means of making high-temperature measurements inclusive of optical pyrometers must be recognized. Measurements obtained by the use of such instruments are not precise, a certain amount of variability being inherent in the instruments themselves, and in the perceptions of different users. (See Fink Patent No. 2,082,622 for a like instance). Moreover, metals are rarely obtainable in a pure state, and those used in industry are known to contain small amounts of other metals and of so-called non-metals. Commercial iron and steel commonly contain carbon, manganese, sulphur, phosphorus, silicon, etc. Nickel (electrolytic as well as that produced in a crucible) contains cobalt, iron and copper. Copper contains some copper oxide. Electrolytic chromium is usually quite pure, but contains some chromium oxide. The noble metals almost invariably contain other of the noble metals along with the principal constituent. The composition of the commercial forms of metals generally is similar.

Moreover, the temperature given in scientific tables for the melting point of a eutectic, varies. For example, in the case of iron and chromium, Adcock, Journal Iron and Steel Institute, London, Sept. 1931, gives the temperature of the melting-point of the eutectic as 1507° C. Von Vegersack, Zeitschrift für Anorganische Chemie, 154, 30 (1926) gives a range of temperatures for the melting-point of the iron-chromium eutectic from 1150° C. when the iron used contains 4% carbon to 1490° C. when the iron used contains practically no carbon. These appear to be the most recent data available.

In practice we use a temperature at or about the melting point of the eutectic, at which a rapid alloying of the constituent metals occurs, while the article maintains its form, with the formation of an alloy layer or band having a definite alloy composition, which temperature is usually within about 50° C. of the temperature of the melting-point of the eutectic given in scientific tables, for eutectics having high melting-points, for example those above 1000° C.

An example of our process is as follows:

An iron wire, or strip, etc., is coated with an electro-deposit of chromium to any desired thickness. Strips and the like may be coated on one or both sides. The coated wire is then heated in the ordinary atmosphere of an electrically heated furnace to a temperature at or somewhat above its eutectic melting point, which lies between 1400° to 1500° C., for 3 to 30 minutes, depending on the thickness of the chromium coating. The heating may also be done in air by electric current passing through the wire or strip.

Another example of our process is as follows:

An iron wire or strip is coated with an electro-deposit of chromium to any desired thickness. The coated wire is then heated in an atmosphere of hydrogen (or in the ordinary atmosphere of a furnace) at a suitable temperature to form a superficial chromium-oxide film on the surface of the chromium coating; for instance, at 1000° to 1200° C. for one to two minutes. The coated article is then transferred to a furnace and heated in an atmosphere of hydrogen (or in the ordinary atmosphere of an electrically-heated furnace)

at a temperature of 1400° to 1500° C. for 3 to 30 minutes, depending on the thickness of the chromium coating. Ordinary commercial hydrogen may be used.

Another example is as follows:

A strip of cobalt is electroformed, and then coated with an electrodeposit of chromium, so that the proportions will be as desired. Alternate layers may be formed. This is then heated to a temperature at or somewhat above its eutectic melting-point, which was between 1400° to 1500° C. A preliminary heating at a lower temperature may be practiced, if desired.

Other examples of our process are as follows:

A nickel wire or strip is coated with an electro-deposit of chromium to any desired thickness. Or an iron wire or strip is coated with an electro-deposit of nickel, or of nickel and chromium, to any desired thickness. These coated wires or strips, etc. are then heated in the manner hereinbefore described. A preliminary heating, as desired or found most suitable, as heretofore described, may be practiced.

If the outermost metal-layer is relatively susceptible to oxidation, an electroplate of a metal which is relatively resistant to oxidation (nickel for example) may be applied before heating. This may be a thin deposit.

Further examples, of alloy sheets, rods, wires, etc., for which the present process may be used advantageously are: Ni—Fe; Pt—Ir; Cr—Ni; Cr—Co; Cr—Fe; W—Cr—Co; W—Cr—Fe; Ni—Cr—Fe; Ni—Fe—Mo. Each of these metals has a melting point above 1000° C. The process is moreover applicable generally to the formation of alloy articles.

A mode of procedure in carrying out our process is illustrated in the accompanying drawing:

An electroformed, or mechanically formed, sheet, strip, rod wire, etc. (iron for example), enters a cleaning bath 10 at *a*; from which it enters a washing bath 11, as indicated at *b*. The sheet, etc., is then electroplated, entering a chromium-plating bath 12 for example, as indicated at *c*. The article may then be given a protective coating (of nickel, for example), and for this purpose may enter a washing bath 13 at *d*, an acid-dip 14 at *e*, and a nickel-plating bath 15 at *f*. It may then enter a washing bath 16 at *g*. If it is desired to form a preliminary superficial oxid film in the article, it may then go into a "low temperature" furnace 17 as indicated at *h*. The article enters the furnace 18 at *i* where it is heated to a temperature at or about the eutectic melting point, or above, to form the alloy. The exit from the furnace 18 is indicated at *k*. The article, as heretofore explained, may enter the furnace 18 directly, and the furnace 18 may contain a non-oxidizing atmosphere, or not, as may be desired or most suitable.

The process may be carried out by other modes of procedure than those herein specifically illustrated and described.

What is claimed is:

1. A process of treating metal articles to alloy constituent metals, which comprises coating a formed metal article with a solid adherent layer of another metal in intimate metallic contact with the first metal, the metals having melting points above 1000° C. and also above the melting point of the eutectic, and forming an alloy of the constituent metals by heating the coated article at a temperature at or about the melting point of the eutectic of the metals, which will produce

rapid diffusion while the article maintains its form.

2. A process of treating metal articles to alloy constituent metals, which comprises coating a formed metal article with a solid adherent layer of another metal in intimate metallic contact with the first metal, the metals having melting points above 1000° C. and also above the melting point of the eutectic, and forming an alloy of the constituent metals by heating the coated article at a temperature at or about the melting point of the eutectic of the metals, which will produce rapid diffusion while the article maintains its form, in a reducing or non-oxidizing atmosphere.

3. A process of treating metal articles to alloy constituent metals, which comprises coating a formed metal article with a solid adherent layer of another metal in intimate metallic contact with the first metal, the metals having melting points above 1000° C. and also above the melting point of the eutectic, heating the coated article to form a superficial oxide film thereon, and thereafter forming an alloy of the constituent metals by heating the coated article at or about the melting point of the eutectic of the metals, which will produce rapid diffusion while the article maintains its form.

4. A process of treating metal articles to alloy constituent metals, which comprises coating a formed metal article with a solid adherent layer of another metal in intimate metallic contact with the first metal, the metals having melting points above 1000° C. and also above the melting point of the eutectic, heating the coated article in a reducing or non-oxidizing atmosphere to form a superficial oxide film thereon, and thereafter forming an alloy of the constituent metals by heating the coated article at or about the melting point of the eutectic of the metals, which will produce rapid diffusion while the article maintains its form.

5. A process of treating metal articles to alloy constituent metals, which comprises coating a formed metal article with a solid adherent layer of another metal in intimate metallic contact with the first metal, the metals having melting points above 1000° C. and also above the melting point of the eutectic, heating the coated article to form a superficial oxide film thereon, and thereafter forming an alloy of the constituent metals by heating the coated article in a reducing or non-oxidizing atmosphere at or about the melting point of the eutectic of the metals, which will produce rapid diffusion while the article maintains its form.

6. A process of treating metal articles to alloy constituent metals, which comprises coating a formed metal article with a solid adherent layer of another metal in intimate metallic contact with the first metal, the metals having melting points above 1000° C. and also above the melting point of the eutectic, heating the coated article to form a superficial oxide film thereon, and thereafter forming an alloy of the constituent metals by heating the coated article at or about the melting point of the eutectic of the metals, which will produce rapid diffusion while the article maintains its form, both heatings being done in an ordinary reducing or non-oxidizing atmosphere which incidentally contains some oxygen.

7. A process according to claim 1, further comprising coating the outermost coat with a coat of a metal less susceptible to oxidation at high tem-

perature, than said outermost coat, prior to heating at said high temperature.

8. A process according to claim 1 wherein the article which is coated is electroformed.

9. In a process of treating metal articles to alloy constituent metals, forming an alloy of the constituent metals by heating a metal article having thereon a solid adherent coating metal in intimate metallic contact with the first metal, the metals having melting points above 1000° C. and also above the melting point of the eutectic, at a temperature at or about the melting point of the eutectic of the metals, which will produce rapid diffusion while the article maintains its form.

10. In a process of treating metal articles to alloy constituent metals forming an alloy of the constituent metals by heating a metal article having thereon a solid adherent coating metal in intimate metallic contact with the first metal to form a superficial oxide film thereon, said metals having melting points above 1000° C. and also above the melting point of the eutectic, and thereafter heating at a temperature at or about the melting-point of the eutectic of the metals, which will produce rapid diffusion while the article maintains its form.

11. In a process of treating metal articles to alloy constituent metals, coating the outermost coat of a coated metal article with a coat of metal less susceptible to oxidation at high temperature than said outermost coat, said metal and coating having melting points above 1000° C. and also above the melting point of the eutectic, and then forming an alloy of the constituent metals by heating at a temperature at or about the melting-point of the eutectic of the metals, which will produce rapid diffusion while the metal maintains its form.

12. In a process of forming ferro-chromium alloy articles, alloying the constituents by heating an article comprising layers of iron and chromium in intimate metallic contact at a temperature at or about the temperature of the melting point of the eutectic, between 1400 to 1500° C. for a relatively short time while the metals rapidly diffuse and the article maintains its form.

13. In a process of forming ferro-chromium alloy articles, according to claim 12, preliminarily heating said article at a lower temperature to develop a thin protective oxid film thereon.

14. In a process of forming ferro-nickel-chromium alloy articles, alloying the constituents by heating an article comprising layers of iron, nickel and chromium in intimate metallic contact at a temperature at or about the temperature of the melting point of the eutectic, above 1400° C. for a relatively short time while the metals rapidly diffuse and the article maintains its form.

15. In a process of forming ferro-nickel-chromium alloy articles according to claim 14, preliminarily heating said article at a lower temperature to develop a thin protective oxid film thereon.

16. In a process of forming alloy articles, alloying the constituents by heating an article comprising layers of metals in intimate metallic contact having melting points above 1400° C. at a temperature at or about the melting point of the eutectic of the metals for a relative short time while the metals rapidly diffuse and the article maintains its form.

COLIN G. FINK.  
PINCUS DEREN.